

## UNITED STATES PATENT OFFICE

CAMILLE DREYFUS AND WILLIAM R. BLUME, OF NEW YORK, N. Y., ASSIGNEES TO  
CELANESE CORPORATION OF AMERICA, A CORPORATION OF DELAWARE

TEXTILE MATERIAL CONTAINING ORGANIC ESTERS OF CELLULOSE AND METHOD OF  
PREPARING THE SAME

No Drawing.

Application filed July 18, 1928. Serial No. 293,781.

This invention relates to the treatment of fabrics or yarns containing organic esters of cellulose in such a manner that the fabrics or yarns may be safely ironed by means of 5 irons or calenders that are at higher temperatures than may safely be employed with previously known textile materials.

An object of our invention is to produce textile material containing organic esters of 10 cellulose that have higher safe ironing temperatures than previously known textile materials of this type. Other objects of our invention will appear from the following detailed description.

15 Textile materials containing yarns of organic esters of cellulose may ordinarily not be ironed with an iron whose temperature is above about 230° C. since the organic esters of cellulose material tends to stick to the 20 iron above this temperature. To increase the safe ironing point of such textile materials, it has been proposed to partially saponify the same, and it has also been proposed to weight these textile materials with 25 metallic salts. In either case, however, the safe ironing point is raised to a predetermined amount, which, in the case of cellulose acetate textile material, does not generally exceed 260° C. We have made the 30 surprising discovery that if textile materials containing organic esters of cellulose are first partially saponified and then weighted with a metallic salt or other weighting agent the safe ironing point of the material is increased considerably, so that these materials 35 may be ironed at temperatures above that at which even cotton or silk scorches. Thus, a fabric containing cellulose acetate yarn, when treated in accordance with our invention, has a safe ironing point of 275° to 285° C. or more.

In accordance with our invention, we partially saponify the textile material, made of or containing organic esters of cellulose by means of an alkaline bath of suitable concentration and at suitable temperatures. The so partially saponified material is then weighted with metallic salts or other weighting agents to the desired degree.

The textile material to be treated in ac-

cordance with our invention may be a woven, knitted or netted fabric or it may be yarn in the form of hanks, or wound on bobbins, cones or other textile packages.

The textile material to be treated may 55 contain any suitable organic ester of cellulose such as cellulose acetate, cellulose formate, cellulose propionate or cellulose butyrate. The textile material may consist wholly of one or more of these organic 60 esters of cellulose, or may be a mixed fabric or yarn containing yarns of these organic esters of cellulose and yarns of cotton, silk or reconstituted cellulose (rayon).

The alkaline bath used for partially saponifying the cellulose acetate contained in the fabric or yarn may be either of low concentration or of high concentration depending on the temperature of treatment. If an alkaline solution of low concentration is 70 used, higher temperatures may be employed in the process, whereas if alkaline solutions of high concentrations are used, low temperatures of treatment are employed. If a solution of intermediate concentration is 75 employed, intermediate temperatures of treatment should be used.

The saponifying bath may contain any suitable alkali or alkaline salt for producing hydroxyl ions in aqueous solutions. Of the 80 alkalies that are suitable, sodium hydroxide, potassium hydroxide or ammonium hydroxide may be mentioned. Examples of alkaline salts are sodium or potassium carbonates, sodium or potassium phenolate, sodium 85 or potassium sulphite, sodium or potassium silicate, or tri-sodium phosphate. In order to promote intense surface saponification of the yarn containing the organic ester of cellulose, buffer salts or modifying agents 90 such as soap, sodium acetate, borax or alcohol, etc. may be added to the saponifying bath.

When alkaline solutions of low hydroxyl concentration are employed, the bath should 95 contain at least 0.2 grams of sodium hydroxide of the equivalent amount of other alkaline substances per liter of solution, when temperatures of 80° C. are employed. While we do not limit ourselves to the specific con- 100

centration, we have found that solutions having a hydroxyl ion content corresponding to 0.4, 0.5, 0.6 or 0.7 grams of sodium hydroxide per liter, give eminently satisfactory results. The temperature of the bath is maintained at 60° to 90° C. and preferably at about 80° C. However, after saponification of the cellulose acetate textile material has been initiated, the saponifying bath may contain less sodium hydroxide, since saponification then proceeds in a bath containing hydroxyl ions in amounts corresponding to less than 0.2 grams of sodium hydroxide per liter. The saponification may proceed to any desired extent, say 3% or 5 to 10% or more. These percentages represent the percent of loss of weight the cellulose acetate has suffered through the saponification treatment.

20 The saponification of the fabric with alkaline solutions of low concentrations may be carried out in a tank, on the jig, on the winch or in any other suitable device. Often it is desirable to thoroughly wet out the fabric prior to subjecting it to the saponification bath. The addition of soap to the saponification bath is of great advantage in promoting level saponification of the organic esters of cellulose material, and also the presence of the soap in the saponifying bath tends to help to cause the saponification to be concentrated on the surface of the yarn containing the organic esters of cellulose, which causes desirable increase in safe ironing point. While the proportions of soap to the solution may be varied within wide limits, it may be stated that the presence of 0.5 grams to 10 grams of soap per liter of solution produces satisfactory results.

45 In one mode of carrying out the partial saponification with the use of solutions containing alkali in low concentrations, the goods are scoured in an open bath on strings or in any suitable machine such as a jig, with a bath containing olive oil soap for an hour or two. The goods may then be removed from the bath and saponified in a separate bath containing fresh water and alkali, but they are preferably saponified directly in the general scouring bath by the addition of a requisite amount of caustic soda. In one mode of partially saponifying the fabric containing the organic ester of cellulose with an alkaline solution of low concentration, the fabric is immersed in a bath of such large volume that it contains sufficient alkali to cause the desired degree of saponification but which is not of such concentration to exceed the maximum permissible concentration of alkali material at the temperature to be employed. Thus for example, in saponifying a fabric consisting wholly of cellulose acetate of approximately 65 54% acetyl value, we have found that a bath

of up to 120 to 180 times the weight of the fabric can advantageously be used, and that such a bath should preferably contain an amount of caustic soda to the extent of 4 to 8% of the weight of the fabric, when a bath temperature of 80° C. is used. Obviously, if the fabric or yarn contains other organic esters of cellulose or an alkaline material other than caustic soda is used or if the temperature of the bath is other than 80° C., the proportions will be varied accordingly. Likewise it is apparent that when smaller amounts of alkaline material are used the volume of the saponification bath may be correspondingly decreased.

75 In another mode of carrying out the saponification when alkaline solutions of low concentrations are employed, the fabric or yarn containing the yarns of cellulose acetate is treated in an alkaline bath of comparatively small volume and containing a relatively small amount of caustic soda. As the saponification proceeds, further quantities of caustic soda are added in small increments, until the desired degree of saponification has taken place. Until the operator has gained sufficient experience, it is preferable to check up the amount of caustic soda in the bath by titration with sulfuric acid to insure that the amount of caustic soda added is not sufficient to cause the saponifying bath to have a concentration exceeding the maximum permissible degree.

95 When concentrated alkaline solutions are used, the concentration of the alkali solution preferably corresponds to from 5 to 20% of caustic soda by weight. To increase the safe ironing temperature, a 20% caustic soda solution is preferred, since by the use of this solution the safe ironing temperature of a cellulose acetate fabric is materially increased. The saponifying bath may also contain such assistants as soap, sodium acetate, etc. The alkali solution may be applied to the fabric containing the organic esters of cellulose in any suitable manner. However, we prefer to apply the caustic soda when applied in comparatively concentrated solution to the fabric by padding the caustic solution onto the fabric and then permitting the same to stand for an appreciable length of time. The temperature of treatment is preferably room temperature and should not exceed 35° C. for obtaining the best results.

105 110 115 120 125 130 The textile material after saponification by any of the above methods, is then weighted by subjecting the same to a swelling agent and a weighting agent. The swelling agent and the weighting agent may be applied in separate baths or they may be applied in the same bath. Furthermore the weighting agent may of itself be a swelling agent so that the use of another swelling agent may not be necessary. Examples of

swelling agents are comparatively concentrated aqueous solutions of acetic acid, formic acid, lactic acid, or acetone. Examples of weighting agents are aqueous solutions of stannic chloride or tannic acid, strong solutions of which are also swelling agents.

5 After treating with the weighting agent, the fabric is subjected to the action of a fixing bath which contains alkaline phosphates or silicates.

10 The product formed by our process has a safe ironing point that is from 10 to 25° C. or more higher than the safe ironing point of the textile materials that have been 15 saponified alone or have been weighted alone. Moreover, the fabric produced by our process has a softer hand than fabrics that have been subjected to the weighting process alone or to the partial saponification 20 process alone.

25 For the best results, the textile material should be first partially saponified and then weighted, rather than first weighted and then partially saponified, since a much higher safe ironing point may be imparted to the textile material by the process that involves first partially saponifying and then weighting. While we do not limit ourselves to this theory we believe that this is due 30 to the fact that if the textile material is first weighted, the presence of the weighting agent causes saponification to proceed throughout the whole fabric, as against the intense surface saponification produced by 35 the partial saponification of the unweighted textile material by the process above described.

40 In order to further illustrate our invention the following detailed example is given, but this invention is not limited thereto.

#### Example

45 A woven fabric consisting wholly of cellulose acetate yarn is plaited and strung, and is then immersed in a bath in which the ratio of water to fabric is between 130 and 160 to 1. This bath contains soap to the extent of 1 gram per liter of bath and the bath temperature is maintained at 80° C. 50 The fabric is treated in this soap bath for three-quarters of an hour. It is then raised out of the bath, and caustic soda in an amount equal to 6% of the weight of the fabric is added to the bath, and after the 55 solution is homogeneous, the fabric is then immersed in the bath and is treated therein for approximately three hours while the bath temperature is maintained at 80° C. The fabric is then lifted and washed off in 60 water at 60° C.

65 The so partially saponified fabric is then weighted as follows. One part of the fabric is treated with 30 parts of a 40° Tw. solution of stannic chloride for one-half hour at 55° to 65° C. The fabric is rinsed

off in water and then treated with a 7° Tw. solution of sodium silicate. The fabric is then washed with or without soap, and is found to have increased in weight by 20%. If desired, this fabric may be dyed or 70 printed.

The safe ironing point of the fabric has been increased by this process by 60° C. or more, as is indicated by the fact that the safe ironing point of the fabric, after it 75 has been treated as above described, is increased to 280° C. to 285° C. The safe ironing point is determined by measuring the maximum temperature of an iron that does not stick to, melt or scorch the fabric 80 when said iron is permitted to rest upon the fabric for five seconds. The safe ironing point of a cotton fabric when tested in this manner is not appreciably over 260° C.

85 It is to be understood that the foregoing detailed description is given merely by way of illustration and that many variations may be made therein without departing from the spirit of this invention.

Having described our invention, what we 90 claim and desire to secure by said Letters Patent is:

1. Method of increasing the safe ironing point of a textile material containing organic esters of cellulose comprising both 95 partially saponifying the organic esters of cellulose and weighting the textile material.

2. Method of increasing the safe ironing point of a textile material containing cellulose acetate comprising both partially saponifying the cellulose acetate and weighting the textile material. 100

3. Method of increasing the safe ironing point of a textile material containing organic esters of cellulose comprising subjecting the textile material to a solution of alkali and then weighting the same. 105

4. Method of increasing the safe ironing point of a textile material containing organic esters of cellulose comprising subjecting the textile material to a solution of alkali and then weighting the same with a tin compound. 110

5. Method of increasing the safe ironing point of a textile material containing organic esters of cellulose comprising subjecting the textile material to a solution of alkali and then weighting the same with a tannic acid compound. 115

6. Method of increasing the safe ironing point of a textile material containing organic esters of cellulose comprising subjecting the textile material to a solution of alkali, then weighting the same by treatment with a tin salt, and then fixing the tin by treatment with a precipitating agent, whereby a textile material having a safe ironing point above 270° C. is produced. 120

7. Method of increasing the safe ironing point of a textile material containing cellulose. 125

lose acetate comprising subjecting the textile material to a solution of alkali and then weighting the same.

8. Method of increasing the safe ironing

5 point of a textile material containing cellulose acetate comprising subjecting the textile material to a solution of alkali and then weighting the same with a tin compound.

9. Method of increasing the safe ironing

10 point of a textile material containing cellulose acetate comprising subjecting the textile material to a solution of alkali, then weighting the same by treatment with a tin salt, and then fixing the tin by treatment

15 with a precipitating agent, whereby a textile material having a safe ironing point above 270° C. is produced.

10. Method of increasing the safe ironing point of a textile material containing cellulose acetate comprising subjecting the textile

20 material to a solution of alkali, then weighting the same by treatment with a tannic acid solution, and then fixing the tannic acid compounds by treatment with a precipitating 25 agent, whereby a textile material having a safe ironing point above 270° C. is produced.

11. A textile material containing partially saponified organic esters of cellulose, which textile material is weighted with a 30 weighting agent.

12. A textile material containing partially saponified cellulose acetate, which textile material is weighted with a weighting agent.

35 13. A textile material containing partially saponified organic esters of cellulose, which textile material is weighted with a tin compound.

14. A textile material containing partially 40 saponified organic esters of cellulose, which textile material is weighted with a tannic acid compound.

15. A textile material containing partially 45 saponified cellulose acetate, which textile material is weighted with a tin compound.

16. A textile material containing partially saponified cellulose acetate, which textile material is weighted with a tin compound, said textile material having a safe ironing 50 point above 270° C.

17. A textile material containing partially saponified cellulose acetate, which textile material is weighted with a tannic acid compound, said textile material having a safe 55 ironing point above 270° C.

18. A textile material containing partially saponified cellulose acetate, which textile material is weighted with a tin compound, said textile material having a safe ironing 60 point between 280° and 285° C.

In testimony whereof, we have hereunto subscribed our names.

CAMILLE DREYFUS.  
WILLIAM R. BLUME.